

# UNITED STATES PATENT OFFICE.

CHARLES C. HUFFMAN, OF CHICAGO, ILLINOIS, ASSIGNOR TO SUNBEAM CHEMICAL COMPANY, OF CHICAGO, ILLINOIS, A CORPORATION OF ILLINOIS.

## UNIVERSAL YELLOW DYE AND METHOD OF PRODUCING THE SAME.

1,274,047.

Specification of Letters Patent. Patented July 30, 1918.

No Drawing.

Application filed September 24, 1917. Serial No. 192,872.

To all whom it may concern:

Be it known that I, CHARLES C. HUFFMAN, a citizen of the United States, and resident of Chicago, in the county of Cook 5 and State of Illinois, have discovered a certain new and useful Universal Yellow Dye and Methods of Producing the Same, of which the following is a specification.

My discovery relates to dyes and particularly to a novel yellow dye having peculiar and advantageous qualities.

I am aware that heretofore dyes have been incorporated in soaps with the object in view of providing a simple carrier for 15 the dye and fairly satisfactory results may be secured if neutral dyes are employed and if the water in which the substance is used is of exactly the right temperature.

My improved dye soap should not be confused with those in which the soap acts merely as a carrier or vehicle for the dye, as the following description will show that the final product is the result of peculiar reactions which take place between the dye 25 and the elements of the soap and which product could not be secured by the use of the materials heretofore employed or as heretofore combined. By reason of the novel process of compounding and the selection of substances which enter into the compound, a dye is produced which is equal if not superior to those which require boiling and the addition of a mordant for setting the color.

One of the important distinctions of the dyes produced by me is that they are alkali proof, irrespective of the characteristics of the dye, that is, basic, neutral or acid, before combining in the soap.

A still further distinction is that the dyes are universal, that is, adaptable to either cotton, wool, silk or flax, or mixtures thereof.

One of the important advantages following the use of the method disclosed is that of allowing the glycerol, which is a by-product of the saponification process, to remain in the product. This is liberated when the soap is dissolved and co-operates 50 with the dye in attacking the fabric. Furthermore it assists in fixing the colors following the application of heat, as in the act of ironing, after the fabric has been dried.

The composition and the method of preparing it will now be described in detail.

In order to establish a basis for the proportions of ingredients, it will be assumed that it is desired to produce five gross of one ounce bars of the soap. To produce this quantity, three gallons and forty-two 60 ounces of vegetable oil and one gallon and twenty-four ounces of sodium hydroxid ( $NaOH$ ) of a specific gravity of 1.40 at 65° F. are combined. The oil or oils used may be varied. Olive, soy bean, raisin, peanut, crude corn, or any vegetable oil may be used separately or combined with cocoanut oil. The proportions of the cocoanut oil and other oils will vary according to weather conditions. Under normal conditions one 70 gallon, fourteen ounces of cocoanut oil will be employed to two gallons, twenty-eight ounces of the other oils. In warm, dry weather the proportion of cocoanut oil should be lessened and increased in cool, 75 damp weather.

The oil and caustic soda are mixed until the saponification is nearly completed at which time the dye solution is added.

I employ chrysoidin, which is an acid 80 azo dye having the formula  $C_6H_5N:N.C_6H_5(NH_2)_2HCl$  and which is normally a dye for producing an orange color. For the production of a universal, alkali proof yellow, a quantity, which will be varied in accordance with the color desired, of chrysoidin is dissolved in one gallon of boiling water and is added to the soap solution shortly before saponification is complete. The addition of this hot solution to the soap, together with the heat of the subsequent reaction, causes the temperature of the bath to be raised to approximately 122° F., at which temperature the excess of sodium hydroxid reacts with the chrysoidin, converting the color acid into its sodium salt;  $C_6H_5N:N.C_6H_5.NaCl.(NH_2)_2$  or sodium diaminoazobenzene chlorid. Apparently, however, this salt is not stable at the temperature described and immediately enters 95 into a new compound in which all traces of the salt as such is obliterated. This theory seems to be confirmed by the fact that the final substance has resisted all efforts to analyze it or to separate the sodium salt of chrysoidin therefrom. The amount of chrysoidin employed for producing a medium yellow will be approximately six ounces 100 105 avoirdupois.

After allowing a few minutes for the re- 110

action to take place and after the dye has become thoroughly mixed with the soap, the soap is poured into molds where it is allowed to remain at a temperature of about 5 80° F. for forty-eight hours.

It will be noted that the glycerol is not removed from the product and therefore will be released as the soap is dissolved. It will be absorbed by the fabric along with the 10 dye and will assist in fixing the dye when heat is applied to the fabric as in ironing. It has furthermore, an advantageous effect on the fabric in softening the same and brightening the colors.

15 In use the soap and the garment or fabric to be dyed are introduced into hot water and the soap may be applied directly to the fabric to thoroughly cleanse the same. Even though the soap is applied locally or 20 only in spots the coloring will be even. Furthermore, the hands or container will not be colored. After the article is cleansed and dyed it is rinsed in cold water and dried in the usual manner. The dye will be found 25 to be alkali proof.

Many other colors are secured by a combination in different proportions of chrysoidin and methylene blue. For instance, green, mustard, citron and other similar 30 colors are produced by dissolving the chrysoidin in two quarts of boiling water and the blue in two quarts of boiling water. At the same stage in the operations, that is, just before saponification of the soap, the 35 chrysoidin solution is added and the reaction allowed to become complete; then the blue solution is added. After this reaction is complete the compound is stirred until there is uniformity and the additional steps 40 are the same as before described. These colors have the same properties as the yellow.

It has been found difficult, if not impossible in prior practice, to combine two 45 colors, particularly an acid and a basic color, without precipitation. By my practice there is no such danger. This feature of my discovery is claimed broadly in a co-pending application.

50 It will be noted that the soap is manufactured by the cold process. By reason of this process of manufacture I am enabled to secure an absolutely uniform product with regard to the colors produced. The low temperatures employed are much more easily controlled and the necessary reaction between the soap and the dye is completed 55 with a certainty which is not possible in a settled soap.

One of the most important features of my 60 novel discovery is that the shade of color which is secured in the use of the article is the same whether a large or small quantity is employed and whether it is used in hot or cold water. It is preferably used with hot 65 water for the reason that the soap will not act to thoroughly cleanse the article unless the water is hot. The effect of deepening the shades by the use of hot water is not present and this is of great importance if 70 it be desired to reproduce certain colors. The ordinary user has no means of determining whether the same temperature is employed in each instance. Neither would he be able to determine whether exactly the 75 same quantity of the dyeing material was employed. By the use of my product the colors may be duplicated with ease and certainty.

By comparison of the proportions of 80 vegetable oil and sodium hydroxid it will be noticed that there is a substantial excess of the latter even when the water containing the dye is added. Of course, the amount of the saponifying agent may be varied somewhat but in any case an excess should be employed.

I claim:

1. The herein described dyestuff composed of the reaction products of a vegetable oil, 90 an excess of a saponifying agent over that required for complete saponification of the oil and chrysoidin, as set forth.

2. The herein described universal dye formed by adding dissolved chrysoidin to a 95 saponified solution containing an excess of a saponifying agent.

3. A universal alkali proof dye chemically combined with soap, the substance being composed of a vegetable oil, an excess of a 100 saponifying agent, and an anilin dye, the product being formed by combining the oil and saponifying agent, then before saponification is complete adding thereto the anilin dye dissolved in water.

4. The method of producing a universal, alkali proof dye combined with a cold process soap, which consists in combining a vegetable oil and an excess of sodium hydroxid, then before saponification is complete adding thereto an anilin dye dissolved in hot water, substantially as described.

Signed at Chicago, Illinois, this 22nd day of September, 1917.

CHARLES C. HUFFMAN.

Witness:

T. D. BUTLER.